# EUROPEAN PATENT APPLICATION

(11) **EP 0 919 637 A1**
(43) Date of publication of application: **02.06.1999**
(21) Application number: 98203029.8
(22) Date of filing: 10.09.1998
(51) Int. Cl.: C22C 38/60, C22C 38/00, C22C 38/40

(54) **Fine-austenite-grain sulphur-containing steel having improved machinability and its method of manufacture**

(30) Priority: 01.12.1997 IT MI972662
(71) Applicant: Lucchini Centro Ricerche E Sviluppo S.r.l., 57025 Piombino (Livorno) (IT)
(72) Inventor: Chioatto, Gianfranco, 20097 San Donato Milanese, (Milan) (IT); Maccio, Giovanni, 57027 San Vincenzo, (Livorno) (IT)
(74) Representative: Appoloni, Romano

(57) **Abstract**

Non-alloy and alloy steels, for case-hardening or quenching and tempering having fine austenitic grains and containing sulphur in the form of spheroidal sulphides of which the values of the spheroidisation index and shape factor are within defined limits.
In the above steels, the combination of well-characterised spheroidal sulphides together with the addition of from 0.05% to 0.30% in weight of bismuth, as an element and/or an alloy and/or as a mixture with one or more elements insoluble in liquid steel or having spheroidizing effects on sulphides, to the liquid-steel ladle or to the mould of a continuous casting machine or tundish of a continuous casting machine, results in a clear-cut improvement of machinability when compared to the existing state of the art. In quantitative terms this improvement of machinability increases cutting-tool life by 70% on average in machining operations, all other cutting parameters and conditions being equal.

## Description

The present invention relates to non-alloy and alloy steels, for case-hardening or quenching and tempering, which have fine grains in the austenitic state, and to the process used to obtain such kinds of steels.

As concerns the production of steels for case-hardening or for quenching and tempering, it has been known for a considerable time that to obtain a definite improvement in machinability, in addition to the traditional steelmaking elements, it is necessary to add lead; tellurium or selenium to to the liquid-steel ladle or to the mould of a continuous casting machine or to the tundish of a continuous casting machine.

However both lead and tellurium are chemical elements which because of their very high toxicity are very harmful to the health of the operators encharged with steelmaking or machining operations.

On the other hand, in the production of steels for case-hardening and/or for quenching and tempering, also sulphur can be used to reduce the toughness of the steel at the tool-chip intertace. Sulphur is normally present in the steel as manganese sulphides which can have various shapes known as type 1 sulphides, type 2 sulphides, type 3 sulphides.

Type 1 sulphides have a spheroidal shape and are obtained in the presence of high oxygen contents (as found in rimming and semi-killed steels for example). Type 2 sulphides have a dendritic structure and separate at the boundaries of the primary grams formed at solidification; these sulphides are formed in killed steels with low aluminium additions which are only just enough to deoxidise the steel. Type 3 sulphides are formed by increasing the quantity of aluminium, or of other elements with a high affinity for oxygen (titanium or vanadium), to reach values sufficient to control austenite grain size.

At the present time, it has been ascertained that spheroidal sulphides are the most suitable for improvement of the machinability of steels for case-hardening or quenching and tempering, because these sulphides are distributed uniformly throughout the steel matrix to form embrittlement and fracture sites for the chip which, in this manner, is broken away more frequently when compared with traditional steels.

Furthermore in high-sulphur steels the spheroidisation of the sulphide incluions significantly diminishes the the worsening of mechanical properties normally associated with the embrittling effect of sulphur. It is known, in fact, that for high sulphur contents and type 2 and 3 sulphide morphologies, the fibre structure of the steel matrix after rolling, characterised by the presence of bands of manganese sulphides in the form of lamellae and stringers aligned along the rolling direction, causes a sharp drop in the energy absorbed by impact-test test-pieces made from samples taken along a direction transverse to that of rolling. When sulphur is present as spheroidal sulphides, the above effect is decidedly attenuated.

However, there is a desire to improve the degree of machinability of fine-austenite-grain non-alloy and alloy steels for case-hardening or quenching and tempering which contain spheroidal sulphides, for it is still low on the whole, especially for specific applications such as machining, with acceptable costs, of components intended for the engineering industry in general and the automotive industry in particular.

The purpose of the present invention is to realise a sulphur-containing steel with fine austenitic gain size having improved machinability and which is not harmful to the health of those who produce it in the steelworks and who subject it to successive hot-working and machining operations.

A further purpose of the present invention is to indicate a method whereby a sulphur-containing steel with improved machinability, as that described herein, can be obtained.

A yet further purpose of the present invention is to realise a sulphur-containing steel with fine austenitic grain size and improved machinability in an inexpensive manner and without employing complex and costly technological means.

These purposes are fulfilled by a sulphur-containing steel with fine austenic grains as in claim 1 and a method of manufacture as in claim 6, reference being made to these claims for the sake of brevity.

The addition of bismuth, as an element and/or as an alloy and/or as a mixture with one or more elements insoluble in liquid steel or having spheroidizing effects on sulphides, in suitable quantities to the liquid-steel ladle or to the tundish or mould of a continuous casting casting machine, such addition being made to sulphur-containing non-alloy and alloy steels, for case-hardening or quenching and tempering, which have fine austenitic grains, has the advantage of permitting the bismuth to be well distributed in a uniform manner in the form of inclusions with dimensions equal to or less than 5 microns.

Attention is drawn above all to the fact that by steels for case-hardening or quenching and tempering having fine austenitic grains are meant steels with such characteristics obtained by the addition of metallic elements such as aluminium, titanium, niobium, vanadium and mixtures of these elements, all of which behave as controllers of austenitic grain size; the total quantity of the above elements introduced into the steel should be equal to or greater than 0.015% in weight for austenitic grain size control.

Furthermore, such steels have sulphur contents in the range from 0.02% to 0.10% in weight. With suitable values of the spheroidisation index and shape factor, the sulphides present in the steel improve machinability when compared to traditional techniques, while ensuring freedom from hot-shortness.
To define the degree of spheroidisation of the sulphides use will here be made of a method based on the relation between the length of the sulphide inclusions in the steel (hereinafter denoted by "ξ") and their thickness (hereinafter denoted by "w").
The so-called "shape factor" of the sulphide inclusions hereinafter denoted by "f" is given by the following formula:${\text{f = P}}^{\text{2}} \text{/(4πA); (f>=1),}$ where P indicates the perimeter of the sulphide inclusions and A indicates their area.

The relation "ξ"/"w" is termed the "spheroidisation index" of the sulphides present in the steel. On the basis of an experimental study on free-cutting steels having only sulphur as an embrittling agent, it was possible to determine the values of the mean statistical spheroidisation index of the sulphides, and their mean statistical shape factor, which gave the best results in machining operations.

It is to be understood that by the term "mean statistical value" used above and hereinafter is meant the determination of the value on a number of samples which is statistically significant, i.e. at least 1 sample per 10 tonnes of steel produced with a minimum number of 3 samples.

The mean statistical value of the spheroidisation index and the shape factor are determined metallographically as follows. Each of the above samples is divided along its longitudinal axis. On one of the sections obtained in this manner, 10 fields, equidistant between the sample axis and one of the longitudinal edges, are selected for examination at a magnification of x200 with an image processor which permits the sulphide morphology to be expressed in quantitative terms.

In order to express in quantitative terms the machinability of steels for case-hardening or quenching and tempering according to the present invention; choice has been made of reference parameters relating to the morphological characteristics of the sulphides, and a machining index hereinafier termed "v20". A range from 0.015 millimetre to 0.20 millimetre (limiting values included) was chosen as the value of the length "ξ" of the sulphide inclusions which appears in the mean statistical index "ξ"/"w".

To determine the value of the machinability index, tests were performed at various cutting speeds within a pre-selected range.Each test lasted for 20 minutes (hence the term "v20" used to indicate this test) and the depth of tool flank wear was measured at the end of the test using appropriate optical instrumentation. Following the indications given up to here, it was posssible to express in quantitative terms the improvement in machinability obtained with type 1 sulphides (lenticular after hot-rolling) compared to type 2 and type 3 sulphides (lamellae or stringers after hot-rolling). This improvement, in terms of the machinability index in turning operations, was found to be 40% on the average. As an example, in the following Table are presented the results of v20 tests, in terms of tool flank wear, performed to determine the values of the machining index for two case-hardening steels (grade 19CrMnS5), one with lamellar sulphides and the other with spheroidal sulphides.

| Test steel/test parameters and data collected | Cutting speed (m/min) Tool flank wear (mm) | Cutting speed (m/min) Tool flank wear (mm) | Cutting speed (m/min) Tool flank wear (mm) | test duration (minutes) |
|---|---|---|---|---|
| ξ/w = 6.00 | 160 - 0.6 (m/min - mm) | 180 - 0.87 (m/min - mm) | 200 - 0.98 (m/min - mm) | 20 |
| f = 2.6 | | | | |
| lamellar sulphides | | | | |
| ξ/w = 4.60 | 160 - 0.37 (m/min - mm) | 180 - 0.44 (m/min - mm) | 200 - 0.67 (m/min - mm) | 20 |
| f = 2.3 | | | | |
| spheroidal sulphides | | | | |

It has already been seen that the addition of manganese to steel ensures freedom from hot-shortness. Type 1 sulphides have a spheroidal structure and are obtained with high oxygen contents; whereas type 2 sulphides (which are formed in steels with low aluminium contents) have a dendritic structure and separate out at the boundaries of the primary grains formed during solidification where they give rise to the hot-shortness effect in steels.

By increasing the quantity of aluminium or other elements (such as titanium and vanadium) up to values that permit austenite grain size to be readily controlled (i.e. to values of more than 0.015% in weight); type 3 sulphides appear which are randomly distributed in the steel with angular irregular shapes.

After hot-rolling, type 1 sulphides have a lenticular shape, whereas type 2 and type 3 sulphides are transformed into platelets or very thin stringers.

As already stated, it is found that a considerably improved degree of machinability results from the presence of type 1 sulphides which have a coarser morphology.

According to the present invention, non-alloy and alloy steels for case-hardening or quenching and tempering are used which contain elements to control austenitic grain size, the contents of said elements being equal to or greater than 0.015% in weight and, in any case, in the range from 0.015% to 0.05% in weight (limiting values included), and which contain from 0.02% to 0.1% in weight of sulphur in the form of spheroidal sulphides which have values of the mean statistical spheroidisation index equal to or less than 4.8 and values of the mean statistical shape factor which are less than or equal to 2.5. The presence of sulphides with values of the spheroidisation index and of the shape factor in the above ranges results in the machinability index being improved by 40% when compared to steels which are identical with the exception of the value of the spheroidisation index which is greater than 4.5 and that of the shape factor which is greater than 2.5.

In addition, according to the present invention, the steels also contain from 0.05% to 0.30% in weight of bismuth (liming values included).

There are no toxicity problems with bismuth which has the added advantage of significantly improving the machinability of steel in a manner comparable to that of lead-containing steels. Lead-containing steels are however extremely dangerous for the operators.

Like lead, bismuth is insoluble both in liquid and solid steel and is distributed as a multitude of particles in the matal matrix, their dimensions normally being less than 5 microns.

The improvement of machinability with bismuth-containing steels is due to the fact that bismuth melts at the temperature reached by the tool and the chip being formed, for the melting temperature of bismuth is 271°C. Bismuth thus acts as an embrittling agent not only in the cutting zone but also in neighbouring zones where the temperature is above the melting temperature of bismuth.

The required doses of bismuth as an element and/or an alloy and/or as a mixture with one or more elements insoluble in liquid steel or having spheroidizing effects on sulphides, are added to the liquid steel in the liquid-steel ladle or mould of a continuous casting machine to obtain, in this manner, a perfect distribution and uniformity of bismuth in the product. There is even more reason to expect such uniformity of distribution if the addition is made to the tundish of a continuous casting machine.

The addition of bismuth as an element and/or as an alloy and/or as a mixture with one or more elements insoluble in liquid steel or having spheroidizing effects on sulphides, to fine-austenite-grain steels, for case-hardening or quenching and tempering, containing spheroidal sulphides with values of the mean statistical spheroidisation index less than or equal to 4.8 and values of the mean statistical shape factor less than or equal to 2.5 results in an average improvement of 70% for the machinability index, whereas the addition of bismuth to steeels with platelet-shaped or stringer-shaped sulphides would lead to an improvement of the machinability index by only 30% on average.
As an example, in the following table are presented the results of v20 tests, in terms of tool flank wear, performed to determine the values of the machining ndex for two case-hardening steels (grade 19CrMnS5), one with lamellar sulphides and the other with spheroidal sulphides plus a bismuth addition.

From the above description are evident the characteristics of the fine-austenite-grain sulphur-containing steel and its method of manufacture, which are subjects of the present invention, as well as the advantages of the said steel.

Finally it is evident that the fine-austenite-grain. sulphur-containing steel for case-hardening or quenching and tempering and its method of manufacture can be subjected to numerous modifications and variations without affecting the innovative nature of the invention, and that in a practical embodiment of the

| Test steel/test parameters and data collected | Cutting speed (m/min) Tool flank wear (mm) | Cutting speed (m/min) Tool flank wear (mm) | Cutting speed (m/min) Tool flank wear (mm) | test duration (minutes) |
|---|---|---|---|---|
| ξ/*w* = 6.00 | 160 - 0.6 (m/min - mm) | 180 - 0.87 (m/min - mm) | 200 - 0.98 (m/min - mm) | 20 |
| f = 2.6 | | | | |
| lamellar sulphides | | | | |
| ξ/*w* = 4.30 | 160 - 0.17 (m/min - mm) | 180 - 0.26 (m/min - mm) | 200 - 0.33 (m/min - mm) | 20 |
| f = 2.1 | | | | |
| spheroidal sulphides and bismuth | | | | |

invention, the materials, shapes, and dimensions of the products can be varied according to need and replaced by other equivalent ones.

## Claims

1. A fine-austenite-grain non-alloy or alloy sulphur-containing steel for case-hardening or quenching and tempering; produced using a continuous-casting machine, the said steel containing sulphur in quantities between 0.02% and 0.1% in weight and a metallic element or elements or mixtures of such elements to control austenite grain size; the steel being characterized by the fact that it contains between 0.05% and 0.30% in weight of bismuth (limiting values included) as an element and/or as an alloy and/or as a mixture with one or more elements insoluble in liquid steel or having spheroidizing effects on sulphides.

2. A steel of claim 1 characterised by the fact that the elements used for austenite grain control are aluminium and/or titanium and/or niobiuim and/or vanadium.

3. A steel of claim 1 characterized by the fact that the elements used for austenite grain control are present individually or as mixtures in quantities which are equal to or greater than 0.015% in weight and, in any case, in the range from 0.015% to 0.05% (limiting values included).

4. A steel of claim 1, characterised by the fact that the bismuth is added, as an element and/or as an alloy and/or as a mixture with one or more elements insoluble in liquid steel or having spheroidizing effects on sulphides, to the liquid-steel ladle or to the tundish of a continuous casting machine or to the mould of a continuous casting machine.

5. A steel of claim 1 characterised by the fact that the sulphur is present in the steel as sheroidal sulphides having a value of the mean statistical spheroidisation index; defined as the relation between the length and thickness of said sulphide inclusions, which is equal to or less than 4.8 in absolute terms, and having a value of the mean statistical shape factor, defined as the relation between the sqaure of the perimeter of said sulphur inclusions and the area of said inclusions multiplied by the product of 4 and π, which is less than or equal to 2.5 in absolute terms, such that it is possible to attain a particularly high and reliable machinability when compared to the present state of the art.

6. A steel of claim 5 characterised by the fact that the said mean statistical spheroidisation index and the mean statistical shape factor are determined on a number of samples which is statistically significant, i.e. at least 1 sample per 10 tonnes of steel produced with a minimum number of 3 samples.
The mean statistical value of the spheroidisation index and the shape factor are determined metallographically as follows. Each of the above samples is divided along its longitudinal axis. On one of the sections obtained in this manner, 10 fields, equidistant between the sample axis and one of the longitudinal edges, are selected for examination at a magnification of x200 with an image processor which permits the sulphide morphology to be expressed in quantitative terms.

7. A method for the production of fine-austenite-grain non-alloy or alloy sulphur-containing steel for case-hardening and/or quenching and tempering which contains from 0.02% to 0.10% in weight of sulphur and which is produced using a continuous casting machine, said method being characterised by the fact of consisting of the following stages:
- addition of sulphur to the steel in quantities between 0.02% and 0.10% in weight in order to obtain spheroidal sulphides the morphology of which is such that that the mean statistical spheroidisation index is less than or equal to 4.8 and the mean statistical shape factor is less than or equal to 2.5.
- addition of aluminium and/or titanium and/or niobium and/or vanadium, or mixtures of such elements, the total quantity of said elements being equal to or greater than 0.015% and, in any case, in the range from 0.015% to 0.05% (limiting values included).
- addition of bismuth, as an element and/or as an alloy and/or as a mixture with one or more elements insoluble in liquid steel or having spheroidizing effects on sulphides, to the liquid-steel ladle or to the tundish of a continuous casting machine or to the mould of a continuous casting machine in quantities between 0.05% and 0.30% (limiting values included).
